

## UNITED STATES PATENT OFFICE.

WILLIAM MENDEL, OF BEVERLY, NEW JERSEY, ASSIGNOR TO SAMUEL A. NEIDICH,  
OF EDGEWATER PARK, NEW JERSEY.

## MANUFACTURE OF ARTIFICIAL SILK FROM VISCOSE.

No Drawing.

Application filed May 28, 1925. Serial No. 33,503.

*To all whom it may concern:*

Be it known that I, WILLIAM MENDEL, a citizen of the United States, residing at Beverly, in the county of Burlington and State of New Jersey, have invented a certain new and useful Improvement in the Manufacture of Artificial Silk from Viscose, whereof the following is a specification.

My invention relates to the manufacture of filaments by projecting viscose (variously known as cellulose sulphocarbonate or cellulose thiocarbonate) through minute spinneret orifices into baths containing chemicals which coagulate the viscose as a semi-solid impure cellulose hydrate, which must be subjected to subsequent cleaning processes and thereafter dried to form the commercial artificial silk.

Natural silk filaments have an average diameter of .015 millimeter and, therefore, it is highly desirable to produce artificial silk filaments of approximately the same diameter. However, the aforesaid coagulated viscose elements must, of course, be of sufficient strength to withstand the stresses of manipulation incident to their production, and as the viscose products of ordinary processes are much weaker and more frangible than the natural silk filaments; it has been found impossible to commercially manufacture viscose silk filaments which are less than double the diameter of the natural silk filaments. For instance, if dried in air, the minimum diameter of ordinary viscose silk filaments is .03051 millimeter and if viscose silk filaments are subjected to the action of glycerine, as is usual to improve their flexibility, the minimum ultimate diameter attainable is .03545 millimeter.

Therefore, an object and effect of my invention is to provide a method and means for commercially producing viscose silk filaments as fine, lustrous and elastic as natural silk filaments.

Various chemicals are used in the precipitating bath aforesaid. For instance, because of their prompt action and relatively low cost, strong acid baths, such as aqueous solutions containing eight per cent of sulphuric acid of five per cent of hydrochloric acid, are commonly used. With baths of that character, substantially all of the sulphur primarily chemically combined with the cellulose in viscose is released as free

sulphur, but is occluded in the mass of cellulose hydrate, causing the latter to present an undesirable dull yellow white appearance, whereas, natural silk has a characteristic lustrous, translucent appearance. Therefore, such ordinary processes of coagulation must be supplemented by successive treatments of the coagulated viscose in chemical baths with a view to removal of the sulphur impurities therefrom. However, although such cleansing operations are only partially successful, they leave the viscose filaments weak, brittle and inelastic as compared with natural silk.

Microscopic examination of such ordinary viscose silk filaments discloses that their inherent weakness as compared with natural silk filaments is due to the fact that whereas, a natural silk filament is of substantially uniform homogeneous solid structure with a smoothly continuous surface; an ordinary viscose filament is of porous structure with a pitted surface; the formation of such pores and pits being incident to the primary inclusion and occlusion of sulphur derivatives in the cellulose hydrate and subsequent partial elimination of the same, leaving the cellulose hydrate of spongy texture.

Therefore, an object and effect of my invention is to provide a method and means for commercially producing viscose silk filaments without occluding free sulphur or its derivatives therein and to thus avoid weakening the coagulated cellulose hydrate filament by the formation of pores and pits as aforesaid, and it is the attainment of that result which permits the formation of filaments, in accordance with this invention, as fine as natural silk filaments.

I have discovered that the desirable results aforesaid are attainable by subjecting viscose to the action of  $\text{PO}_4$  ions. Such ions have a beneficial effect if added to or formed in the viscose, or in any bath in which viscose may be coagulated, or in a fluid distinct from either the viscose or the coagulating medium and, in the latter case, may be either alone or in association with other matter affecting the viscose complex. For instance, the impure cellulose hydrate product of coagulation of viscose may be subjected to  $\text{PO}_4$  ions in a fluid containing dyeing material or detergent material.

$\text{PO}_4$  ions have the apparent effect of preventing the formation of sulphur or its

derivatives in insoluble form, and thus render the coagulated products practically self-cleansing. However, if  $\text{PO}_4$  ions be added to or formed in the viscose before coagulating the same in the form of filaments, they have the effect of accelerating the progressive "aging" of the viscose which is manifested by progressive increment in viscosity of the viscose which may or may not be desirable in accordance with the process of coagulation to which the viscose is to be subjected. However, in the form of my invention herein contemplated, I prefer to subject the viscose to the action of  $\text{PO}_4$  ions in a bath in which the viscose is coagulated in the form of filaments; so that the aforesaid aging effect of the  $\text{PO}_4$  ions upon the uncoagulated mass of viscose is avoided, but the viscose filament is beneficially affected by the  $\text{PO}_4$  ions immediately upon introduction to the bath, and thus immediately strengthened to withstand the stresses to which it is subjected, in its progression through and from the bath.

Such  $\text{PO}_4$  ions may be added to or produced in such coagulating baths in any convenient form or manner. However, tri-sodium phosphate ( $\text{Na}_3\text{PO}_4$ ) is a cheap vehicle for such ions and is further preferable because it may be conveniently used in aqueous solution.

Although an aqueous solution of either mono-sodium phosphate or di-sodium phosphate, or said tri-sodium phosphate alone will effect coagulation of viscose projected therein, particularly if the viscose is of low alkalinity and such solution be hot; even a small percentage, approximating a mere trace of the ion  $\text{PO}_4$ , is sufficient in association or conjunction with any other suitable coagulating material. The beneficial effect of employing even a minute quantity thereof is so great as to warrant the inference that its effect is what is termed "catalytic".

For instance, an aqueous bath containing 10 per cent of sulphuric acid, ( $\text{H}_2\text{SO}_4$ ) and containing 10 per cent of sodium sulphate ( $\text{Na}_2\text{SO}_4$ ) is an ordinary coagulating bath which is subject to the objections aforesaid, but I find that the addition of even a fraction of 1 per cent of  $\text{PO}_4$  to such bath has the advantageous results above contemplated, in the elimination of, or prevention of formation of, insoluble sulphur derivatives in or upon the filaments projected therein.

However, I prefer to use an aqueous solution containing sodium bi-sulphite ( $\text{NaHSO}_3$ ) and salammoniac (ammonium chloride  $\text{NH}_4\text{Cl}$ ), for instance, containing twenty-five per cent of the former and ten percent of the latter. Such a bath promptly coagulates the viscose to an impure cellulose hydrate complex sufficiently coherent to be mechanically drawn through and from such

bath over a roller. However, unless  $\text{PO}_4$  ions are present during the reactions incident to coagulation of viscose in such a bath, the resulting product contains the objectionable free sulphur and its derivatives above contemplated. Therefore, I include such ions in said bath, conveniently in the initial form of tri-sodium phosphate ( $\text{Na}_3\text{PO}_4$ ) in aqueous solution, say, three per cent. However, it is to be understood that the result may be attained with a much lower percentage of  $\text{PO}_4$  ions, as I have found, in some instances, even after prolonged use of such a bath for the coagulating operation above contemplated, the bath contains substantially the amount of  $\text{PO}_4$  ions originally introduced therein and, as above noted, even a fraction of one per cent is sufficient for the purpose herein contemplated.

Filaments thus coagulated in accordance with my invention may require no subsequent treatment other than rinsing with water, as they are practically self-cleansing, in such coagulating bath, and emerge therefrom of substantially uniform homogeneous structure and with smooth surfaces. When such filaments are dried, preferably under tension, they have unusually high luster, strength and elasticity, and filaments even finer than natural silk may be thus produced.

Therefore, I do not desire to limit myself to the precise details of structure, arrangement or procedure herein set forth, as it is obvious that various modifications may be made therein without departing from the essential features of my invention, as defined in the appended claims.

I claim:

1. The method of manufacturing artificial silk filaments from viscose which consists in coagulating viscose by projecting a fine filament thereof into an aqueous solution containing  $\text{PO}_4$  ions.

2. The method of manufacturing artificial silk filaments from viscose which consists in coagulating viscose by projecting a fine filament thereof into an aqueous solution containing  $\text{PO}_4$  ions associated with other ions capable of affecting such coagulation.

3. The method of manufacturing artificial silk filaments from viscose which consists in coagulating viscose by projecting a fine filament thereof into an aqueous solution containing  $\text{PO}_4$  ions associated with other ions capable of effecting such coagulation and including sodium bi-sulphite ( $\text{NaHSO}_3$ ) and ammonium chloride ( $\text{NH}_4\text{Cl}$ ).

4. The method of manufacturing artificial silk filaments from viscose which consists in coagulating viscose by projecting a fine filament thereof into an aqueous solution containing  $\text{PO}_4$  ions associated with other ions capable of effecting such coagulation and in-

cluding sodium bi-sulphite ( $\text{NaHSO}_3$ ) to the amount of twenty-five per cent and ammonium chloride ( $\text{NH}_4\text{Cl}$ ) to the amount of ten percent.

5. The method of manufacturing artificial silk filaments from viscose which consists in coagulating viscose by projecting a fine filament thereof into an aqueous solution containing  $\text{PO}_4$  ions, resultant from inclusion of 10 tri-sodium phosphate ( $\text{Na}_3\text{PO}_4$ ) in such solution.

6. The method of manufacturing artificial silk filaments from viscose which consists in coagulating viscose by projecting a fine filament thereof into an aqueous solution containing  $\text{PO}_4$  ions, resultant from inclusion of 15 tri-sodium phosphate ( $\text{Na}_3\text{PO}_4$ ) in such solution, with another solute capable of effecting such coagulation.

20 7. The method of manufacturing artificial silk filaments from viscose which consists in coagulating viscose by projecting a fine filament thereof into an aqueous solution containing  $\text{PO}_4$  ions, resultant from inclusion of 25 tri-sodium phosphate ( $\text{Na}_3\text{PO}_4$ ) in such solution, with another solute capable of effecting such coagulation.

8. The method of manufacturing artificial silk filaments from viscose which consists in 30 coagulating viscose by projecting a fine filament thereof into an aqueous solution containing  $\text{PO}_4$  ions, resultant from inclusion of tri-sodium phosphate ( $\text{Na}_3\text{PO}_4$ ) in such

solution, with another solute capable of effecting such coagulation in association with 35 a third solute capable of effecting such coagulation.

9. The method of manufacturing artificial silk from viscose which consists in projecting filaments of the latter into an aqueous 40 solution in which tri-sodium phosphate ( $\text{Na}_3\text{PO}_4$ ) has been dissolved, with an acid solute capable of effecting such coagulation.

10. The step in the manufacture of artificial silk which consists in projecting a filament of viscose (thiocarbonate) through an orifice less than .025 millimeter in diameter, 45 into an aqueous bath containing  $\text{PO}_4$  ions and capable of coagulating cellulose hydrate from viscose with release of soluble sulphur derivatives.

11. The step in the manufacture of artificial silk which consists in projecting a filament of viscose (thiocarbonate) through an orifice less than .025 millimeter in diameter, 55 into an aqueous bath containing  $\text{PO}_4$  ions and capable of coagulating cellulose hydrate from viscose with release of soluble sulphur derivatives; such solution being resultant from mixture of water with an inorganic acid and tri-sodium phosphate ( $\text{Na}_3\text{PO}_4$ ). 60

In testimony whereof, I have hereunto signed my name at Burlington, New Jersey, this 20th day of May, 1925.

WILLIAM MENDEL.